

Aug. 11, 1970

K. H. J. BUSCHOW ET AL  
PERMANENT MAGNET CONSTITUTED OF FINE PARTICLES  
OF A COMPOUND  $M_5R$

Filed Jan. 19, 1968

3,523,836

2 Sheets-Sheet 1



FIG. 1

INVENTOR.  
K. H. J. BUSCHOW  
W. A. J. J. VELGE

BY

Frank R. Jifan  
AGENT

Aug. 11, 1970

K. H. J. BUSCHOW ET AL  
PERMANENT MAGNET CONSTITUTED OF FINE PARTICLES  
OF A COMPOUND  $M_5R$

3,523,836

Filed Jan. 19, 1968

2 Sheets-Sheet 2



FIG. 2

INVENTOR.  
K. H. J. BUSCHOW  
W. A. J. J. VELGE

BY

Frank R. Jurgens

AGENT

## 1

3,523,836

### PERMANENT MAGNET CONSTITUTED OF FINE PARTICLES OF A COMPOUND $M_5R$

Kurt Heinz Jürgen Buschow and Wilhelmus Antonius Johannes Josephus Velge, Emmasingel, Eindhoven, Netherlands, assignors, by mesne assignments, to U.S. Philips Corporation, New York, N.Y., a corporation of Delaware

Continuation-in-part of application Ser. No. 644,101, June 7, 1967. This application Jan. 19, 1968, Ser. No. 699,232

Claims priority, application Netherlands, Jan. 21, 1967, 6700998

Int. Cl. C22c 19/00, 31/00; H01f 1/06

U.S. Cl. 148—31.57

4 Claims

#### ABSTRACT OF THE DISCLOSURE

A permanent magnet is constituted of a body composed of fine particles of a compound  $M_5R$  in which M is cobalt or a combination of cobalt and one of the metals Fe, Ni or Cu and R is  $La_{1-x}Ce_x$  where  $0 < x < 1$ .

This application is a continuation-in-part of application Ser. No. 644,101, filed June 7, 1967.

The invention relates to a permanent magnet constituted of fine particles having in themselves permanent magnetic properties. The component of these particles which is essential to these magnetic properties is  $M_5R$  where R is a combination of the two rare earth elements La and Ce, and M is either Co or a combination of Co with one or more of the elements Fe, Ni and Cu.

In the prior application permanent magnets are disclosed, the component of which is essential to the permanent magnetic properties is  $M_5R$  where M is cobalt or a combination of cobalt and one of the metals Fe, Ni and Cu and R is La, Th with a earth metal, or at least three rare earth metals. Such magnets have a high uniaxial anisotropy combined with a high saturation magnetization.

Permanent magnets also are required to have both a high saturation moment  $\sigma$ , and a high intrinsic coercive force,  $IH_C$ .

According to the invention a permanent magnet as described in the previous application has a component essential to the permanent magnetic properties a compound  $M_5R$ , R, however, now is  $La_{1-x}Ce_x$ .

Such a permanent magnet, according to the invention, may in particular have an  $IH_C$  of more than 3500 oersteds (oe.) combined with a  $\sigma$  of more than 30 erg/gauss oersted (g.oe.) when  $0 < x < 0.6$ .

When  $0.2 < x < 0.6$  a combination of  $IH_C > 3500$  oe. and  $\sigma > 90$  (g.oe.) are reached.

The invention will be described with reference to the accompanying drawing, the sole figure of which shows the dependence of  $IH_C$  and  $\sigma$  as functions of  $x$ .

Graph 1 shows how, in a permanent magnet constituted of fine particles of compounds of the series  $La_{1-x}Ce_xCo_5$ ,  $0 < x < 1$ , the value of  $IH_C$  depends upon  $x$ .

The  $IH_C$  values plotted in this graph are always the highest obtained values of a particular compound in the series. The  $IH_C$  measured actually depends upon the size of the particles measured. By reducing these particles in

## 2

size so that they increasingly show a "single-domain-character," the  $IH_C$  increases in principle. However, the reduction of the particles in size also involves a deformation. This may just have an opposite effect in various cases on the value of  $IH_C$ ; however the  $IH_C$  values from which Graph 1 was plotted have all been measured with an experimentally determined optimum average particle size.

Graph 2 shows the variation of the saturation magnetization  $\sigma$  also as a function of  $x$  for the same series of compounds.

It is found that the values of both  $IH_C$  and  $\sigma$  for  $0 < x < 1$  differ substantially from what might be expected from what is known for these quantities for  $x=0$  and  $x=1$ . With a suitable choice of  $x$  the manufactured permanent

15 magnets may show combinations of  $\sigma$  and  $IH_C$  which are more favorable than those of the permanent magnets constituted of the compounds for which  $x=0$  or  $x=1$ .

These magnets are made using the process described in the aforesaid application Ser. No. 644,101, viz., a body is

20 first manufactured by melting the component elements to form the compound of  $M_5R$  and subsequently the mass is cooled. The body is if necessary homogenized by annealing in an atmosphere which protects against oxidizing influence at a temperature just below the melting point. After being cooled to room temperature the body is pulverized and the powder molded into a body in a magnetic field.

While the invention has been described with reference to specific embodiments, other modifications will be apparent to those skilled in this art without departing from the spirit and scope of the invention which is defined in the appended claims.

What is claimed is:

1. A permanent magnet constituted of a body composed of fine particles having in themselves permanent magnetic properties and which consist of a compound  $M_5R$ , M being selected from the group consisting of Co and a combination of Co with at least one of the elements selected from the group consisting of Fe, Ni and Cu and R is  $La_{1-x}Ce_x$ ,  $0 < x < 1$ .

2. A permanent magnet as claimed in claim 1 in which M is Co.

3. A permanent magnet as claimed in claim 1 in which  $0 < x < 0.6$ , said magnet having an  $IH_C$  exceeding 3500 oe. and  $\sigma$  exceeding 30 erg./g.-oe.

45 4. A permanent magnet as claimed in claim 1 in which  $0.2 < x < 0.6$ , said magnet having an  $IH_C$  exceeding 3500 oe. and  $\sigma$  exceeding 90 erg./g.-oe.

#### References Cited

##### UNITED STATES PATENTS

- |                                          |         |                  |       |          |
|------------------------------------------|---------|------------------|-------|----------|
| 2,813,789                                | 11/1957 | Glaser           | ----- | 75—123   |
| 3,102,002                                | 8/1963  | Wallace et al.   | ----- | 75—152 X |
| 3,326,637                                | 6/1967  | Holtzberg et al. | ----- | 75—152 X |
| 3,342,591                                | 9/1967  | Gambino et al.   | ----- | 75—152   |
| 3,421,889                                | 1/1969  | Ostertag et al.  | ----- | 75—170   |
| 3,424,578                                | 1/1969  | Strnat et al.    | ----- | 75—213   |
| 60 L. DEWAYNE RUTLEDGE, Primary Examiner |         |                  |       |          |
| G. K. WHITE, Assistant Examiner          |         |                  |       |          |
| U.S. Cl. X.R.                            |         |                  |       |          |
| 75—152, 170; 148—101, 103                |         |                  |       |          |